

W. F. BLEECKER.  
PROCESS OF REDUCING TUNGSTIC OXIDE TO TUNGSTEN METAL.  
APPLICATION FILED JULY 8, 1920.  
1,427,187. Patented Aug. 29, 1922.



INVENTOR.  
*W.F. Bleecker*

BY  
*John J. Melechner*  
ATTORNEY.

# UNITED STATES PATENT OFFICE.

WARREN F. BLEECKER, OF BOULDER, COLORADO, ASSIGNOR TO THE TUNGSTEN PRODUCTS COMPANY, OF BOULDER, COLORADO, A CORPORATION OF COLORADO.

## PROCESS OF REDUCING TUNGSTIC OXIDE TO TUNGSTEN METAL.

1,427,187.

Specification of Letters Patent. Patented Aug. 29, 1922.

Application filed July 8, 1920. Serial No. 394,630.

To all whom it may concern:

Be it known that I, WARREN F. BLEECKER, a citizen of the United States, residing at Boulder, in the county of Boulder and State 5 of Colorado, have invented certain new and useful Improvements in Processes of Reducing Tungstic Oxide to Tungsten Metal, of which the following is a specification.

This invention relates to a method of reducing tungstic oxide to tungsten metal and its primary object is to provide a simple, efficient and practical process which avoids the difficulties encountered in the usual process of reducing tungstic oxide by the application 15 of heat exteriorly of receptacles in which it is contained.

Inasmuch as the reduction proceeds from the outside inwardly molecule by molecule until the entire mass is reduced, the old 20 process is extremely slow, it being apparent that it would be impractical to pack the material in layers sufficiently thin to provide for a more rapid permeation of the heat required for reduction.

25 In the present process as will hereinafter be described in detail, the heat is applied interiorly of a mass of oxides to be reduced, in the presence of a suitable carbonaceous reducing agent and is compelled to permeate 30 uniformly through the mass by the provision of voids or ducts through which the gases of reduction may pass to a point of escape.

By this method a mass of oxides is heated 35 rapidly and uniformly by a continuous circulation of heat in all directions from an interior point of radiation.

The tungstic oxid may be obtained by any of the well-known methods at present in use, 40 although I prefer to employ the granular product of the process of producing tungstic oxid from sodium tungstate described in my application for patent, Serial No. 387,670 filed June 9, 1920, and allowed May 7, 1921.

45 In this process the tungstic oxide is obtained by mixing a moist sodium tungstate with an amount of sulphuric acid, heating the mixture for the formation of tungstic oxide and sodium sulphate, and removing 50 the sulphate and other soluble salts by proper washing. The result of this process is a practically insoluble tungstic oxide in granular form, particularly well adapted for use in producing metallic tungsten by the 55 present process.

In carrying out my process I employ an electric furnace of suitable construction of either the conductive heat, reflecting arc or resistance type.

A furnace specially constructed for use in carrying out the process has been shown in longitudinal section in the accompanying drawings, and in the following description reference will be had thereto by the use of numerical characters of reference.

60 The furnace shown in the drawings embodies an arcing or heating chamber 2 below a reduction chamber 3 from which it is separated by a carbon or graphite partition 4 upon which the charge is supported.

65 The partition is preferably made of carbon or graphite rods spaced apart to provide passages for the gases developed in the heating chamber, and the reduction chamber is normally closed by a roof 8 which is removed to charge the furnace.

70 The chambers have linings of a nonconductive material, that of the heating chamber being preferably composed of electrically fused magnesite and that of the reduction chamber of ground coke or graphite 75 rammed in place.

75 Two electrodes 5 extending oppositely into the heating chamber through water-cooled openings in the wall thereof are spaced apart to form a jumping gap for the arc by which the material is heated.

80 The tungstic oxid to be reduced to metallic tungsten is mixed with a preferably carbonaceous reducing agent either before or after it is placed in the furnace.

85 The reducing agent may be a solid carbonaceous material such as finely ground coke, coal, charcoal or wood, a reducing gas such as hydrogen, carbon-monoxide, methane, gasoline or kerosene vapors or water gas, or a mixture of both.

90 In case a solid reducing agent is used, the tungstic oxid and the carbonaceous material are thoroughly mixed and the mixture 95 placed in the reducing chamber of the furnace or in using a gaseous reducing agent the tungstic oxid is placed in the reducing chamber without preliminary preparation and the gas is introduced into the charge of 100 the furnace through one or more tubes passing through the wall of the structure in connection with a conveniently placed source of supply.

105 In either case the charge of tungstic oxid 110

with or without the reducing agent is packed in the reduction chamber of the furnace either in the form of briquets or by means of suitable ramming forms.

- 5 Irrespective of the reducing agent used the spaces of gas voids are made throughout the charge to permit of a continuous circulation of heat and gases of reduction while the process is carried on. The spaces 10 or gas voids may be produced either by the use of metal rods which are removed as soon as the charge is packed in the furnace, by distributing a number of small wooden rods throughout the charge which are consumed as soon as the mass is heated and thus provide voids, or by providing the furnace with a series of tubes made of carbon or some highly refractory fused substance such as silica or alundum which are placed in an up- 15 right position throughout the charge in the reduction chamber in connection with the heating chamber below the same.

In the first two constructions the heat and gases or reduction passing through the voids 20 will enter the porous mass at any point thereof, whereas in the last-mentioned construction the gases must necessarily rise in the metal tubes and then work downwardly through the mass.

25 30 The tubes in this case function more as conductors of heat than as a means for applying a gaseous reducing agent.

In the drawing the reference numeral 6 designates the charge of tungsten oxide, 7 35 the wooden or metal rods or tubes disposed therein, and 10 a tube for the introduction of gas into the charge.

Another method of producing the voids 40 consists in mixing the mass with a combustible material such as sawdust, shavings or small pieces of wood which during the progress of the process are consumed and thereby increase the porosity of the charge.

45 In case the material in the reduction chamber is loosely packed, the means for the production of artificial voids may be omitted.

After the furnace has been charged by any 50 of the above-described methods, and its roof 8 is replaced, and luted so as to leave a small vent 9 for the escape of various gases or reduction, the electric circuit in which the electrodes are connected is closed to produce an arc in the heating chamber of the furnace.

55 60 The heat thus produced circulates rapidly through the voids in the charge of the reduction chamber and slowly brings the mass to the reduction temperature, the gases acting upon the reduction agent are reduced and then acting upon the tungsten oxids re-

From this it will be understood that reduction takes place through the medium of gas or vapors which are present in the furnace rather than by actual contact of particles of tungstic oxide and carbon.

65 In using a solid reducing agent such as coke the theoretical amount thereof, plus an excess of from 5 to 10% is mixed with the 70 granular oxides after the coke has been ground to the desired fineness.

The reduction takes place at a temperature somewhat above the critical reduction 75 temperature of tungsten trioxide (approximately 1100 degrees C.) requiring as a maximum a current of 600 amperes and 70 volts. Either alternating or direct current may be used and an electrical resister, either solid or granular, may be employed in the place of 80 the electrodes if so desired.

A suitable binder, molasses for example, 85 may be mixed with the charge to prevent the material at certain stages of deoxidization from crumbling and running under the arc 90 thereby causing dust and consequent loss of material.

95 It has been found that during the process sulphur contained in the tungstic oxides is volatilized to such an extent as to render the finished metal sufficiently low in sulphur to meet the most exacting technical requirements and in order to obtain the maximum elimination of sulphur, care must be taken that as little iron as possible is entered into 100 the material by contact with iron utensils or apparatus, or other causes.

What I claim and desire to secure by Letters Patent is:

1. The herein described method of reducing tungstic oxides to metallic tungsten consisting in applying heat interiorly of a mass of tungstic oxides in the presence of a suitable reducing agent, said mass having artificially produced voids or passages for the 105 circulation of gases.

2. The herein described method of reducing tungstic oxides to metallic tungsten consisting in interspersing combustible matter in a mass of tungstic oxides to produce artificial voids or passages for the circulation of 110 gases, and applying heat interiorly of said mass in the presence of a suitable reducing agent.

3. The herein-described method of reducing tungstic oxides to metallic tungsten consisting in heating a mixture of sodium tungstate and sulphuric acid to produce tungstic oxides and sodium sulphate and applying heat interiorly of the tungstic oxides 115 120 in the presence of a reducing agent.

In testimony whereof I have affixed my signature.

WARREN F. BLECKER.